

Jan. 15, 1957

J. H. EDWARDS ET AL

2,777,775

PRODUCTION OF ARTIFICIAL FILAMENTS, THREADS, AND THE LIKE

Filed May 13, 1954



FIG. 1.



FIG. 2.

# United States Patent Office

2,777,775

Patented Jan. 15, 1957

2,777,775

## PRODUCTION OF ARTIFICIAL FILAMENTS, THREADS, AND THE LIKE

John Harold Edwards and Ernest Edward Tallis, Coventry, England, assignors to Courtaulds Limited, London, England, a British company

Application May 13, 1954, Serial No. 429,640

Claims priority, application Great Britain June 25, 1953

1 Claim. (Cl. 106—165)

This invention relates to the production of artificial filaments, threads, fibres and the like hereinafter referred to as filaments, from viscose.

It is known that viscose filaments produced by the normal spinning processes have a crenulated surface and a structure which consists of a skin and a core. This skin and core effect can be demonstrated by staining a cross-section of the filaments under specific conditions with selected dyestuffs. In addition to the difference in dyeing affinity and in swelling property between the skin and core, the cellulose molecules of the skin are believed to be more highly orientated than those of the core.

The object of the present invention is to obtain modified viscose filaments which have a skin substantially thicker than is normally obtained.

According to the present invention a process for the production of artificial filaments comprises extruding viscose containing at least 0.1 millimole per 100 grams of viscose of a diaryl thiourea having the general formula



where  $R_1$  and  $R_3$  are hydrogen or aliphatic or aryl radicals and  $R_2$  and  $R_4$  are aryl radicals, into an aqueous coagulating bath containing sulphuric acid, sodium sulphate and zinc sulphate.

The preferred minimum concentration for addition to the viscose is one millimole per 100 grams of viscose and the preferred maximum concentration is 10 millimoles per 100 grams of viscose. The filaments obtained have a skin substantially thicker than normal and by adjusting the amount of the diaryl thiourea added filaments with non-crenulated surfaces are obtained. The cross-sectional shape and the crenulation of the surface of the filaments is dependent on the particular diaryl thiourea being used and the quantity added to the viscose. Tests may be necessary in order to determine the quantity of diaryl thiourea necessary to give a desired cross-sectional shape and a surface free from crenulations. The coagulating bath preferably contains from  $\frac{1}{2}$  to 15 percent of zinc sulphate.

The present invention also includes viscose containing at least 0.1 millimole per 100 grams of the viscose of a diaryl thiourea having the general formula



wherein  $R_1$  and  $R_3$  are hydrogen or aliphatic or aryl radicals and  $R_2$  and  $R_4$  are aryl radicals.

2

The preferred diaryl thiourea for use according to the present invention is thiocarbanilide  
( $C_6H_5NH—CS—NHC_6H_5$ ).

5 In addition to the non-crenulated surface and the substantial increase in skin thickness the filaments obtained by the process of the invention have a lower water imbibition than unmodified viscose filaments and they have a reduced gel swelling factor.

10 When extruding viscose according to the process of the present invention the distance from the jet at which the thread becomes neutralised is considerably increased by the presence of a diaryl thiourea in the viscose. The process of the present invention enables unripened or so-called "green" viscose to be spun.

15 The invention is illustrated by the following example, in which the percentages are by weight.

### Example

20 Viscose containing 7.4 percent of cellulose, 7.0 percent of caustic soda and 1.1 percent of combined sulphur was prepared in the usual manner. 1.0 millimole per 100 grams of viscose of thiocarbanilide was added and the viscose was mixed for one hour. When the viscose was 48 hours old from the beginning of the mixing stage and had a salt figure of 5.7 it was ready for spinning.

25 This viscose was extruded through a jet having 750 holes, each 0.003 inch in diameter, into an aqueous coagulating bath containing 9.5 percent of sulphuric acid, 20 percent of sodium sulphate and 4.5 percent of zinc sulphate to give a thread of 1550 denier and 750 filaments.

30 The length of immersion in the bath was 24 inches and the temperature of the bath was 48° C. The thread was drawn from the bath at a rate of 28 metres per minute by

35 a godet and then passed through a dilute sulphuric acid bath maintained at a temperature of 95° C. to a second godet rotating at a higher speed than the first godet, to impart an 80 percent stretch to the thread. The thread was collected in a centrifugal spinning box rotating at

40 4000 revolutions per minute. The cake obtained was washed free from acid, a suitable finish was applied and the cake was dried.

45 The filaments had a non-crenulated surface and the filaments were bean shaped in cross-section. The amount of skin was at least 50 percent greater than the amount found in filaments spun under identical conditions without the addition of the thiocarbanilide to the viscose. Moreover the boundary between the skin and core was very diffuse.

50 Filaments prepared in the manner described above and filaments from unmodified viscose were stained to demonstrate the skin and core effect using the technique described in the Textile Research Journal, 1945, page 443.

55 In the accompanying drawings Figure 1 shows stained cross-sections of filaments from unmodified viscose and Figure 2 the stained cross-sections of filaments spun in the presence of thiocarbanilide.

The bean shaped cross-section, thick skin and diffuse boundary between skin and core of the filaments of Figure 2 contrasts with the substantially circular cross-section, crenulated surface, thin skin and sharp boundary between the skin and core of the unmodified filaments of Figure 1.

What we claim is:

60 Viscose containing at least 0.1 millimole per 100 grams of the viscose of thiocarbanilide.

### References Cited in the file of this patent

#### UNITED STATES PATENTS

- |           |           |               |
|-----------|-----------|---------------|
| 2,118,293 | Brinker   | May 24, 1938  |
| 2,322,981 | Ubbelohde | June 29, 1943 |
| 2,435,295 | Stasse    | Feb. 3, 1948  |